

# UNITED STATES PATENT OFFICE.

JACOB BARAB, OF DOVER, NEW JERSEY, ASSIGNOR TO HERCULES POWDER COMPANY, OF WILMINGTON, DELAWARE, A CORPORATION OF DELAWARE.

## NITROGLYCOLS.

1,307,033.

Specification of Letters Patent. Patented June 17, 1919.

No Drawing.

Application filed July 24, 1918. Serial No. 246,453.

*To all whom it may concern:*

Be it known that I, JACOB BARAB, a citizen of the United States, residing at Dover, county of Morris, and State of New Jersey, 5 have invented a new and useful Improvement in Nitroglycols, of which the following is a full, clear, and exact description.

It has been known for years that the glycols, such as ethylene, butylene and propylene, are 10 capable of nitration to produce explosives analogous in their properties to nitroglycerin, and such capacity might be said to be quite obvious in view of the analogous character of glycol and glycerin. Equally 15 obvious, of course, is the possibility of nitrating any mixture of glycols. However, until comparatively recently, the possibilities in this direction have been of only academic interest, because of the impossibility 20 of producing glycols on an economical and commercial scale. Efforts have been made to produce these glycols by cracking oil gas, chlorinating the unsaturated derivatives to chlorhydrins, and making the glycols 25 from the chlorhydrins. The chlorination of these unsaturated derivatives to chlorhydrins presented, for some time, apparently insuperable difficulties. Bringing them in contact with chlorin gas in any 30 known way resulted, so far as any measure of success was attained, in the production of dichlorids, or so-called "Dutch liquid," which could not be successfully converted to glycol. Within a comparatively recent 35 period, however, successful processes have been developed for the chlorination to chlorhydrin of certain of the olefins on a commercial scale, and thus, for the first time, the possibilities of nitrating glycols derived 40 from these olefin chlorhydrins began to assume a practical importance.

It has been assumed that the usual processes in general use for the manufacture of nitroglycerin from glycerin could be applied 45 unchanged to the manufacture of nitroglycol from glycol, but my own exhaustive experiments demonstrated that thereby no explosive could be thus produced that would in any sense meet commercial requirements. 50 Thus, in the purification of the material after nitration, the washing alternately with water and sodium carbonate was found not

to be practicable and it was discovered that it was essential to avoid the use of sodium carbonate. I eventually succeeded, however, in nitrating propylene glycol, and my preferred process for so doing is set forth in an application filed by me July 14, 1917, Serial No. 181,561. This propylene glycol dinitrate possesses certain qualities which, in the literature of the art, have been ascribed to nitrated glycols generally or which might have been taken for granted by a chemist possessing ordinary theoretical knowledge of the subject, but it exhibited 60 other qualities without which it would hardly have been available as a substitute for nitroglycerin; and I believe the disclosures of my said application were the first in the art to give such information with respect to the manufacture of a nitroglycol as would enable those skilled in the art to make the explosive without the necessity of independent experimentation. Among the valuable qualities of propylene glycol dinitrate, 65 aside from its very low freezing point, are its relative insensitiveness to friction and shock as demonstrated by the hammer test, its non-hygroscopicity, its very high boiling point, its stability above the highest range 70 of atmospheric temperature, its gradual evaporation without explosion when subjected to a gradual elevation of temperature to an exceedingly high point, its decomposition without exploding when dropped into 75 a flame, and its endurance of the Abel heat test at 71° C. for a prolonged period.

There are certain objections to propylene glycol dinitrate that by no means offset its advantages or constitute a real hindrance 80 to its practicable use but which, if they could be removed even in degree, would enhance the practical value of the explosive. Thus it is much more volatile at atmospheric temperatures than nitroglycerin. Again, its 85 oxygen balance is comparatively low, there being a deficiency of about 29% as compared with the oxygen required to secure ideal conditions of combustion. This deficiency may readily be supplied by adding an oxygen carrier. Thus, when absorbed in wood pulp or other absorbent carrier, the addition of sodium nitrate, as in the manufacture of dynamite, raises the oxygen balance to the 90 100

desired point. However, it is obvious that it is desirable, if possible, to produce a nitroglycol whose oxygen balance, without the addition of an oxygen carrier, will be relatively high.

Nitrated butylene glycol fails to meet the requirements. Its oxygen balance is much lower than that of nitrated propylene glycol and its volatility is very high.

10 I have made exhaustive experiments with ethylene glycol and have found that the nitrated product possesses qualities analogous to those of nitrated propylene glycol. Thus, like nitrated propylene glycol, when heated 15 in a capillary tube, it burns without explosion, it is stable at the highest range of atmospheric temperature, and it gradually evaporates without explosion when subjected to a gradual elevation of temperature to an 20 exceedingly high point. In certain respects, however, it is not comparable in value to nitrated propylene glycol. Thus, the freezing point of nitrated ethylene glycol is about 25  $-18^{\circ}$  to  $-19^{\circ}$  C. On the other hand, the freezing point of nitrated propylene glycol is so low that I have not been able to determine it. Upon cooling, no viscosity was observable until about  $-48^{\circ}$  C. was reached, and even at  $-77^{\circ}$  C., while the mass was 30 quite stiff, it had not solidified. Nitrated ethylene glycol cannot, therefore, be said to be non-freezing at atmospheric temperatures. In severely cold weather, it would be necessary, in its manufacture, to warm it to 35 prevent freezing. It would possess no practical advantage over nitroglycerin in any climate where below zero (Fahrenheit) temperature is prevalent.

Again, nitrated ethylene glycol cannot 40 compare with nitrated propylene glycol with respect to sensitiveness to shock or friction. It is much less sensitive to shock or friction, however, than nitroglycerin, although, when subjected to a severe hammer test, it explodes, like nitroglycerin, whereas propylene glycol dinitrate does not.

Nitrated ethylene glycol, however, has the 45 advantage over nitrated propylene glycol of having no deficiency in oxygen and the secondary advantage of being less volatile.

Nitrated butylene glycol possesses no advantages over either of the other two nitrated products, but its disadvantages are so pronounced that its practical use can hardly 50 be given serious consideration. Thus, even nitrated propylene glycol and nitrated ethylene glycol are volatile as compared with nitroglycerin, but the volatility of nitrated butylene glycol is much higher than either 55 of the other two nitroglycols; and its oxygen deficiency is far greater than that of nitrated propylene glycol.

The above experiments have led to the discovery that an explosive superior to propylene glycol dinitrate can be produced by the

addition thereto of ethylene glycol dinitrate in various proportions, say from 40 to 60 per cent. of each, or by nitrating a mixture of the two glycols. The explosive possesses the distinct advantage over nitrated propylene glycol of having a much higher oxygen balance and a somewhat lower volatility. While the freezing point is much higher than that of nitrated propylene glycol, it is still so low as to warrant its designation as 70 a non-freezing explosive. With approximately equal proportions of the two nitrated products, the freezing point would be in the neighborhood of  $-40^{\circ}$  C. I prefer to employ from 40 to 50 per cent. nitrated ethylene glycol and from 50 to 60 per cent. nitrated propylene glycol. The proportion of the former should not be less than 35 per cent. or above 60 per cent., while the proportion of the latter should not be less than 40 80 per cent. or above 65 per cent.

An unexpected quality of the new explosive is that it possesses a strength greater than that of either of its constituent explosives.

It is quite practicable to mix the two glycols and nitrate them together. The procedure may be the same as in the manufacture of nitroglycerin with the following modifications: In view of the lower specific 90 gravity of the glycols, more vigorous agitation is required. While to nitrate 100 pounds of ethylene glycol requires 203 pounds of nitric acid and to nitrate 100 pounds of glycerin requires 205 pounds of nitric acid, to 95 nitrate an equal weight of propylene glycol requires only 166 pounds of nitric acid. A mixture of ethylene and propylene glycols also requires substantially less nitric acid 100 than does glycerin. 100 pounds of a mixture of 35 per cent. ethylene glycol and 65 per cent. propylene glycol require 179 pounds of nitric acid. Instead of washing with water and sodium carbonate solutions, as in the purification of nitroglycerin, the washing 110 should be with water and weak ammonia solutions. Any substantial quantity of sodium carbonate in the washing solution is distinctly harmful. If the two glycols are nitrated separately, I prefer to use the weak 115 ammonia solution only in the washing of the nitrated propylene glycol, and use only pure water in washing the nitrated ethylene glycol. The specific process set forth in my said application may be advantageously 120 used. No difficulty in stabilizing the product is encountered if it be thoroughly washed.

A distinctive advantage in nitrating the mixed glycols is that it is more economical to 125 convert a mixture of olefins to chlorhydrin and then reduce to glycol than to chlorinate propylene and ethylene separately and make a pure glycol from each. The mixture of these two glycols is therefore a cheaper prod- 130

uct than either of the pure glycols, so that my new explosive is both cheaper than, and superior to, nitrated propylene glycol.

It is important, however, if the pure chlor-

- 5 hydrins or pure glycols are not obtained separately and afterward mixed and nitrated, that the mixture of chlorhydrins or mixture of glycols should not contain, in substantial proportions, butylene chlorhydrin or butylene glycol. So far as butylene glycol is present in the mixture of glycols to be nitrated, it is an impurity. The presence of a negligible percentage of the butylene derivatives (say one or two per cent.)
- 10 is not a serious matter, but if present in a substantial proportion, it so increases the volatility of the final product, besides seriously impairing its qualities in other respects, that the explosive is not only distinctly inferior to nitrated propylene glycol, but would be commercially unacceptable.

When absorbed in any of the usual absorbents employed in the manufacture of dynamite, the new explosive, like nitrated propylene glycol, retains all its valuable qualities, and is non-exuding under general conditions of use.

Notwithstanding the insensitiveness to friction of the solid explosive, it can be detonated satisfactorily by means of a weak primer.

The new explosive used in admixture with nitroglycerin and the mixture of nitroglycols and nitroglycerin may be absorbed in any of the standard absorbents for nitroglycerin. For example, when added to nitroglycerin, it lowers the latter's process freezing point and reduces its sensitiveness to heat, friction and shock.

Another valuable quality of the liquid explosive is that it forms a colloid when mixed with nitrocellulose and the resultant gelatin explosive has valuable properties distinguishing it from nitroglycerin gelatins. A

satisfactory composition comprises 14 parts 45 of nitrocellulose (showing 12.25 per cent. nitrogen) and 100 parts of nitrated propylene and ethylene glycol.

The new explosive may also be used in admixture with nitro-compounds, as, for example, trinitrotoluol or trinitrotoluol oils.

Having now fully described my invention, what I claim and desire to protect by Letters Patent is:

1. A nitroglycol explosive composed practically entirely of nitrated propylene and ethylene glycol.

2. An explosive containing a substantial proportion of nitrated glycol derived from oil gas, said nitrated glycol being composed practically entirely of nitrated propylene and ethylene glycol.

3. A nitroglycol explosive containing a substantial proportion of nitrated glycol derived from oil gas, said nitrated glycol being composed practically of nitrated propylene and ethylene glycol; from 35 to 60 per cent. of said nitrated glycol being nitrated ethylene glycol and from 40 to 65 per cent. of said nitrated glycol being nitrated propylene glycol.

4. A nitroglycol explosive composed practically entirely of nitrated propylene and nitrated ethylene glycol each in the proportion of between 40 and 60 per cent. of the whole.

5. An explosive comprising a substantial proportion of nitrated glycol derived from oil gas, said nitrated glycol being composed practically entirely of nitrated propylene and ethylene glycol, in which the amount of nitrated propylene glycol exceeds the amount of nitrated ethylene glycol by not more than 33½ per cent.

In testimony of which invention, I have hereunto set my hand, at Kenil, N. J., on this 17 day of July, 1918.

JACOB BARAB.